

H. LABHARDT,  
PROCESS OF PRODUCING ALKALI METALS,  
APPLICATION FILED DEC. 14, 1914.

1,191,799.

Patented July 18, 1916.



Witnesses:  
William Miller  
Chris H. Almhardt

Inventor  
Hans Labhardt  
By his Attorneys  
Hauff & Barland.

# UNITED STATES PATENT OFFICE.

HANS LABHARDT, OF MANNHEIM, GERMANY, ASSIGNOR TO BADISCHE ANILIN & SODA FABRIK, OF LUDWIGSHAFEN-ON-THE-RHINE, GERMANY, A CORPORATION.

## PROCESS OF PRODUCING ALKALI METALS.

1,191,799.

Specification of Letters Patent. Patented July 18, 1916.

Application filed December 14, 1914. Serial No. 877,099.

To all whom it may concern:

Be it known that I, HANS LABHARDT, citizen of the Swiss Republic, residing at Mannheim, Germany, have invented new 5 and useful Improvements in the Process of Producing Alkali Metals, of which the following is a specification.

During the production of alkali metal by the electrolysis of molten anhydrous hydroxids, hydroxyl ions are liberated at the anode and combine according to the equation:—



15 giving rise to water and oxygen. This water rapidly diffuses through the electrolyte, the diffusion being assisted by the evolution of gas at the anode, and reacts with a part of the alkali metal which has been liberated at 20 the cathode, so that a part of this alkali metal is reconverted into alkali hydroxid, and hydrogen is evolved according to the equation:—



25 Consequently, the yield of alkali metal is diminished.

I have found that I can obtain a much better yield of alkali metal during the electrolysis of molten alkali hydroxids if I replace the alkali, which surrounds the anode and has taken up water, by a fresh quantity of anhydrous caustic alkali. This replacement is preferably carried out continuously, 35 so that a continuous current of fresh anhydrous caustic alkali is supplied to the anode space while the alkali which contains water is run off and can be dehydrated and used over again.

40 This invention can be employed in the electrolysis of single alkali hydroxids, or of mixtures of alkali hydroxids.

The process according to this invention can be carried out, for example, in a cell the 45 upper space of which is separated by one, or more than one, wall dipping slightly into the electrolyte and dividing the said upper space into two, or more, spaces, one of which receives the products liberated at 50 the cathode, namely alkali metal and hydrogen, while another serves as the anode space and collects the oxygen. The electrodes face one another in the electrolyte below the said separating wall, or walls, and can, if 55 desired, have a wire net interposed between

them. A pipe leading to the cell on the cathode side serves for the introduction of dehydrated alkali, while another pipe, situated on the anode side is used for leading away alkali which has absorbed the water, 60 so that the cell is traversed by a current of alkali in the direction from the cathode to the anode. In this way, the alkali which contains water is prevented, (or to a great degree prevented) from traversing from the 65 anode to the cathode space. The current of alkali is regulated so that it is not sufficient to drag with it the rising drops of alkali metal, which metal collects on the surface of the alkali in the cathode space and can 70 be caused to run off continuously, or it can be bailed off from time to time.

Another example of a suitable way of carrying out the process according to this invention is to introduce the fresh anhydrous alkali through an opening at the lower part of the cell and draw off the alkali which contains water from both the anode space and the cathode space, the flow of alkali in the two directions through the cell 75 being regulated by means of valves, or taps, situated in the pipes through which the alkali is led away from the cell.

The drawing accompanying this specification is schematic and represents in vertical section an apparatus suitable for carrying out the process of my invention.

In the drawing A represents the wall of the cell, B is the anode, C is the cathode and D is a wall dipping below the surface of 90 the electrolyte and dividing the upper space into two parts. Oxygen is led away through the pipe E and any hydrogen which may be formed through the pipe F. Fresh molten alkali is passed into the cell through the 95 pipe G, while alkali which has absorbed water at the anode passes away from the cell through the pipe H. The alkali metal which is formed is run off through the pipe K.

100 Now what I claim is:—

1. In the process of producing alkali metal by the electrolysis of molten caustic alkali, the step which consists in passing fresh anhydrous alkali into the cell and removing from the cell alkali which has absorbed water at the anode.

2. In the process of producing alkali metal by the electrolysis of molten caustic alkali, the step which consists in continu- 110

ously passing fresh anhydrous alkali into the cell and continuously removing from the cell alkali which has absorbed water at the anode.

5 3. In the process of producing a mixture of sodium and potassium metal by electrolyzing a mixture of the hydroxids of said metals, the step which consists in continuously passing a fresh anhydrous molten  
10 mixture of the hydroxids into the cell and

continuously removing from the cell a mixture of the hydroxids, which has absorbed water at the anode.

In testimony whereof I have hereunto set my hand in the presence of two subscribing <sup>15</sup> witnesses.

HANS LABHARDT.

Witnesses:

ARTHUR DENONVILLE,  
H. MERLE COCHRAN.